



US010947610B2

(12) **United States Patent**  
**Verma et al.**

(10) **Patent No.:** **US 10,947,610 B2**  
(45) **Date of Patent:** **Mar. 16, 2021**

(54) **MOORING CHAINS COMPRISING HIGH MANGANESE STEELS AND ASSOCIATED METHODS**

(71) Applicant: **ExxonMobil Upstream Research Company**, Spring, TX (US)

(72) Inventors: **Neerav Verma**, Deer Park, TX (US); **Andrew J. Wasson**, Spring, TX (US); **Hyun-Woo Jin**, Easton, PA (US); **Haiping He**, Tomball, TX (US)

(73) Assignee: **ExxonMobil Upstream Research Company**, Spring, TX (US)

(\*) Notice: Subject to any disclaimer, the term of this patent is extended or adjusted under 35 U.S.C. 154(b) by 5 days.

(21) Appl. No.: **16/541,662**

(22) Filed: **Aug. 15, 2019**

(65) **Prior Publication Data**

US 2020/0063245 A1 Feb. 27, 2020

**Related U.S. Application Data**

(60) Provisional application No. 62/720,709, filed on Aug. 21, 2018.

(51) **Int. Cl.**

**B63B 21/20** (2006.01)  
**C22C 38/38** (2006.01)

(Continued)

(52) **U.S. Cl.**

CPC ..... **C22C 38/38** (2013.01); **B63B 21/20** (2013.01); **B63B 21/50** (2013.01); **C22C 38/001** (2013.01);

(Continued)

(58) **Field of Classification Search**

CPC ..... B63B 21/20; B63B 2021/203

See application file for complete search history.

(56)

**References Cited**

**U.S. PATENT DOCUMENTS**

4,428,781 A 1/1984 Norstrom  
8,752,361 B2 6/2014 Smeets et al.  
(Continued)

**FOREIGN PATENT DOCUMENTS**

GB 2132963 A \* 7/1984  
KR 101654684 9/2016

**OTHER PUBLICATIONS**

E. Fontaine, Seawater Corrosion of Ropes & Chain (SCORCh), Oct. 20, 2008, AMOG Consulting, [http://www.fpsoresearchforum.com/JIP\\_Docs/Proposal\\_SCORCH\\_Rev0.pdf](http://www.fpsoresearchforum.com/JIP_Docs/Proposal_SCORCH_Rev0.pdf).

*Primary Examiner* — Sunil Singh

(74) *Attorney, Agent, or Firm* — Bruce M. Bordelon; Leandro Arechederra, III

(57)

**ABSTRACT**

Mooring chains used in offshore environments are typically formed from carbon steels due to their wear and fatigue resistance properties. Although carbon steels may exhibit robust mechanical properties, they are susceptible to corrosion, which can shorten the usable working lifetime of mooring chains, particularly in a seawater environment. Austenitic steels comprising high percentages of manganese may have comparable mechanical properties to the carbon steels commonly used in mooring chains, yet exhibit less susceptibility to corrosion. Austenitic steels suitable for use in mooring chains and other structures in contact with or exposed to a seawater environment may comprise: 0.4-0.8 wt. % C, 12-25 wt. % Mn, 4-15 wt. % Cr, a non-zero amount of Si<3 wt. %, a non-zero amount of Al<0.5 wt. %, a non-zero amount of N<0.1 wt. %, <5 wt. % Mo, and balance Fe and inevitable impurities.

**17 Claims, 4 Drawing Sheets**



(51) **Int. Cl.**  
*C22C 38/06* (2006.01)  
*C22C 38/02* (2006.01)  
*B63B 21/50* (2006.01)  
*C22C 38/00* (2006.01)

(52) **U.S. Cl.**  
CPC ..... *C22C 38/02* (2013.01); *C22C 38/06* (2013.01); *B63B 2021/203* (2013.01); *B63B 2021/505* (2013.01)

(56) **References Cited**

U.S. PATENT DOCUMENTS

|              |    |         |               |
|--------------|----|---------|---------------|
| 2001/0024621 | A1 | 9/2001  | Leppanen      |
| 2003/0167659 | A1 | 9/2003  | Raines        |
| 2007/0107808 | A1 | 5/2007  | Bauk et al.   |
| 2008/0240970 | A1 | 10/2008 | Eto et al.    |
| 2012/0160363 | A1 | 6/2012  | Jin et al.    |
| 2014/0261918 | A1 | 9/2014  | Jin et al.    |
| 2017/0088910 | A1 | 3/2017  | Jin et al.    |
| 2017/0312861 | A1 | 11/2017 | Jin et al.    |
| 2017/0312862 | A1 | 11/2017 | Wasson et al. |
| 2017/0349983 | A1 | 12/2017 | Jin et al.    |
| 2018/0021895 | A1 | 1/2018  | Wasson et al. |

\* cited by examiner



FIG. 1



FIG. 2



FIG. 3



FIG. 4A



FIG. 4B



FIG. 4C



FIG. 4D



FIG. 4E

## 1

**MOORING CHAINS COMPRISING HIGH MANGANESE STEELS AND ASSOCIATED METHODS**

**CROSS REFERENCE TO RELATED APPLICATIONS**

This application claims the priority benefit of United States Provisional Patent Application No. 62/720,709 filed Aug. 21, 2018, entitled MOORING CHAINS COMPRISING HIGH MANGANESE STEELS AND ASSOCIATED METHODS.

**FIELD**

The present disclosure relates to mooring chains having corrosion and fatigue resistance.

**BACKGROUND**

Offshore platforms and related offshore structures have been used for a variety of purposes in the energy industry including recovery of natural resources such as oil and gas, wind power generation, and the like. Early offshore structures were rigid and extended completely from the water surface to the benthic floor (earthen surface) below. More recently, floating offshore structures have been developed, particularly for use in deep water or hostile environments. Floating offshore structures may include, for example, spar platforms, single column floater (SCF) platforms, tension leg platforms, floating storage and offloading vessels (FSO vessels), drilling ships, offshore wind turbines, and the like.

Mooring chains are used to secure various types of floating offshore structures to the earthen surface below the water line. Over their lifetime, mooring chains experience considerable motion-induced stress and may be susceptible to accumulated fatigue damage. Various grades of carbon steel are commonly used materials for fabricating mooring chains, due to the high mechanical strength, toughness, and wear and fatigue resistance offered by this class of materials. Carbon steels commonly used in mooring applications include grades R3, R3S or R4, as defined by the International Association of Classification Societies (IACS-6th revision, 2016). The classification of a given carbon steel as belonging to one of these grades is based upon various characterizations of strength.

Mooring chains may be used in various aquatic environments, but some environments may be more challenging than are others from an engineering and design standpoint. Seawater environments, in particular, can place mooring chains at risk for corrosion, which may necessitate heightened attention to engineering considerations during the design stage of an offshore structure. Corrosion may be particularly problematic when it exacerbates accumulated fatigue or wear damage, but it may also be challenging in its own right even without other types of damage being present.

Both uniform thinning (i.e., general corrosion) and localized pitting may occur upon a steel mooring chain in a seawater environment. Although the design phase of a moored offshore structure may attempt to account for an anticipated rate of corrosion, it is not uncommon to find corrosion rates that are considerably higher (e.g., 2-6 times than anticipated) during field deployment. In addition, it is not straightforward to account for and/or predict pitting corrosion during the design phase, and such corrosion effects are usually not quantitatively taken into account when engineering an offshore structure. Moreover, corrosion rates

## 2

may vary at different locations along the length of a mooring chain (e.g., depending upon whether a given location is submerged or in a periodic splash zone, or the particular subsurface conditions to which the mooring chain is exposed). Accordingly, a generous safety margin for anticipated mooring chain corrosion rates is generally made during the design phase of an offshore structure.

The consequences of excessive corrosion in the mooring chains of an offshore structure can be significant, both from a safety and cost standpoint. Mooring chain corrosion can be a particularly significant safety and cost issue for offshore oil and gas structures. Many moored offshore structures, such as oil platforms, can have working lifetimes measured in dozens of years, whereas their associated mooring chains may have much shorter working lifetimes due to excessive corrosion and wear, particularly when a higher than expected corrosion rate is experienced. In some cases, preemptive replacement of mooring chains may need to take place in the field in order to provide a reasonable operational safety margin. However, field replacement of mooring chains is frequently not a straightforward matter, and replacement costs can easily reach into the tens of millions of dollars or more, not including the cost of the replacement mooring chain itself. Excessive over-engineering of a mooring chain during the design phase of an offshore structure can likewise lead to an undesirable cost burden.

Although various grades of carbon steel may afford mooring chains having acceptable mechanical performance (e.g., IACS R3, R3S and R4 grades), these materials may exhibit undesirably high corrosion rates, particularly in a seawater environment. In addition, hydrogen embrittlement may sometimes be problematic for these carbon steels, both during the manufacturing phase as well as in field use. To account for excessive corrosion rates, mooring chains employing carbon steel may have significantly larger dimensions than would otherwise be required, thereby increasing material costs and chain weights. Beyond a certain size threshold, mooring chains may be difficult to fabricate with the carbon steels conventionally in use, and excessive chain weights may present an operational challenge during field deployment. In some cases, coatings have been applied to carbon steel mooring chains to address excessive corrosion rates, but the applied coatings may add undesirable cost and complexity to an offshore project. In addition, coated chains must be handled carefully during installation to avoid damaging the coating, which may be difficult to accomplish in an offshore environment.

**SUMMARY**

In various embodiments, the present disclosure provides mooring chains comprising: a plurality of links comprising an austenitic steel, the austenitic steel comprising: 0.4-0.8 wt. % C, 12-25 wt. % Mn, 4-15 wt. % Cr, a non-zero amount of Si<3 wt. % Si, a non-zero amount of Al<0.5 wt. % Al, a non-zero amount of N<0.1 wt. % N, <5 wt. % Mo, and balance Fe and inevitable impurities.

**BRIEF DESCRIPTION OF THE DRAWINGS**

The following figures are included to illustrate certain aspects of the present disclosure, and should not be viewed as exclusive embodiments. The subject matter disclosed is capable of considerable modifications, alterations, combinations, and equivalents in form and function, as will occur to one of ordinary skill in the art and having the benefit of this disclosure.

FIG. 1 shows a chart displaying Charpy V-Notch (CVN) impact toughness testing data for Alloys 1-3 of the present disclosure.

FIG. 2 shows a chart displaying ASTM G99 pin and disk average mass loss measurements for Alloys 1-3 of the present disclosure and Comparative Alloy 4 in a synthetic seawater environment.

FIG. 3 shows a chart displaying steady state corrosion data for Alloys 1-3 of the present disclosure and Comparative Alloys 4 and 5 in a synthetic seawater environment.

FIGS. 4A-4E show corresponding cyclic polarization curves for Alloys 1-3 of the present disclosure and Comparative Alloys 4 and 5 in a synthetic seawater environment.

#### DETAILED DESCRIPTION

The present disclosure generally relates to austenitic steels having a good combination of mechanical properties and corrosion resistance and, more specifically, mooring chains comprising a plurality of links formed from the austenitic steels.

As discussed above, carbon steels are commonly used in applications requiring robust mechanical properties, such as in the mooring chains for floating offshore structures. Unfortunately, some carbon steels are susceptible to excessive corrosion in certain environments, such as during continuous or periodic exposure to seawater, as well as hydrogen embrittlement. Excessive corrosion of carbon steels may necessitate premature replacement of mooring chains or other steel components exposed to seawater environments, oftentimes at prohibitively high replacement costs.

The present disclosure provides austenitic steels that may be utilized to form mooring chains and other structures having advantageous properties for continuous or periodic exposure to seawater environments. Namely, the austenitic steels of the present disclosure have mechanical properties meeting or exceeding those of the carbon steels commonly used in mooring chains (e.g., IACS R3, R3S and R4 grades), as well as significantly enhanced resistance to corrosion and hydrogen embrittlement. As such, the austenitic steels disclosed herein may allow mooring chains to be fabricated such that they have longer working lifetimes in the field and/or feature smaller chain dimensions than possible with the carbon steels currently in use while maintaining a comparable engineering safety factor. Both of these features may decrease life cycle costs and/or material costs. In addition, lower mooring chain weights may be realized to afford easier deployment in the field in some cases. Further, the austenitic steels of the present disclosure feature ready weldability using butt welding techniques commonly used for forming chain links with other types of steel. A still further advantage of the austenitic steels disclosed herein is that they are much less susceptible to hydrogen embrittlement compared to ferritic carbon steels having similar mechanical properties. The low susceptibility of the austenitic steels of the present disclosure toward hydrogen embrittlement is believed to be due to the low rate of hydrogen diffusion resulting from the austenitic microstructure, in contrast to the behavior of ferritic carbon steels having high strength. The low susceptibility toward hydrogen embrittlement allows mooring chains with higher strength to be prepared, again resulting in decreased life cycle costs and improved working lifetimes.

The austenitic steels of the present disclosure feature relatively high concentrations of manganese (Mn) to afford the foregoing combination of good mechanical properties and corrosion resistance. Such steel compositions may be

referred to herein as “high-manganese steels.” High-manganese steels for other applications are known for providing high tensile strength and wear performance, which has resulted in these steels historically being used for applications such as railroad frogs (common crossings) and switches, mining applications, rock crushers, and treads for tractors in abrasive environments. More recently, high-manganese steels have been developed for incorporation in slurry-carrying pipelines, such as those used in oil sands production. Advantageously, the austenitic steels of the present disclosure maintain the characteristic strength and wear resistance properties of other high-manganese steels while also exhibiting corrosion resistance through strategic incorporation of other components (alloying elements). For example, additional corrosion resistance properties may be provided to the austenitic steels of the present disclosure by the incorporation of chromium (Cr) and nitrogen (N) in concentrations and under processing conditions that do not appreciably impact the mechanical properties.

Before describing the austenitic steels of the present disclosure in further detail, a listing of terms follows to aid in better understanding the present disclosure.

All numerical values within the detailed description and the claims herein are modified by “about” or “approximately” with respect to the indicated value, and take into account experimental error and variations that would be expected by a person having ordinary skill in the art. Unless otherwise indicated, room temperature is about 25° C.

As used in the present disclosure and claims, the singular forms “a,” “an,” and “the” include plural forms unless the context clearly dictates otherwise.

The term “and/or” as used in a phrase such as “A and/or B” herein is intended to include “A and B,” “A or B,” “A”, and “B.”

For the purposes of the present disclosure, the new numbering scheme for groups of the Periodic Table is used. In said numbering scheme, the groups (columns) are numbered sequentially from left to right from 1 through 18, excluding the f-block elements (lanthanides and actinides).

The term “corrosion resistance” refers to a material’s susceptibility to deterioration caused by exposure to a reactive or corrosive environment.

The term “toughness” refers to a material’s resistance to crack initiation and propagation.

The term “yield strength” refers to a material’s ability to bear a load without deformation.

The term “tensile strength” refers to the strength corresponding to the maximum load carrying capability of a material in units of stress when the failure mechanism of the material is not linear elastic fracture.

The terms “austenite” and “austenitic” refer to a steel metallurgical phase having a face-centered cubic (FCC) atomic crystalline structure.

The terms “martensite” and “martensitic” refer to a steel metallurgical phase that may be formed by diffusionless phase transformation, in which a parent steel (typically austenite) and one or more product phases have a specific orientation relationship.

The term “E-martensite” refers to a specific form of martensite having a hexagonal close-packed atomic crystalline structure which forms upon cooling or straining of an austenite phase. The E-martensite may be formed as close-packed (111) planes of the austenite phase.

The term “ $\alpha$ -martensite” refers to a specific form of martensite having a body-centered cubic (BCC) or body-centered tetragonal (BCT) atomic crystalline structure

which forms upon cooling or straining of an austenite phase. The  $\alpha'$ -martensite may be formed as platelets.

The term "carbide" refers to a compound of carbon with iron or another metal.

The term "nitride" refers to a compound of nitrogen with iron or another metal.

The term "carbonitride" refers to a compound of carbon and nitrogen with iron or another metal.

Unlike ferritic carbon steels, the microstructures of the high-manganese steels disclosed herein feature an austenite phase having a face centered cubic (fcc) structure at room temperature. The austenite phase may be metastable in some instances. According to various embodiments, the austenitic steels of the present disclosure may comprise: 0.4-0.8 wt. % C, 12-25 wt. % Mn, 4-15 wt. % Cr, a non-zero amount of Si less than 3 wt. % Si, a non-zero amount of Al less than 0.5 wt. % Al, a non-zero amount of N less than 0.1 wt. % N, less than 5 wt. % Mo, and balance Fe and inevitable impurities. The term "a non-zero amount" refers to a concentration above that of a manufacturing impurity (inevitable impurities) for a particular component in the austenitic steels of the present disclosure. The non-zero amount may represent a quantity of the component that is intentionally added to a mixture when forming the austenitic steels. It is to be appreciated that the level of manufacturing impurities suitable for characterizing the concentration of a particular component as non-zero may vary for different components (elements) and from composition to composition.

Metastable austenite phases in the austenitic steels of the present disclosure can undergo a number of different phase transformations through strain induction. These transformations may include, but are not limited to, austenite phase transformation into one or more of a microtwinned (fcc) structure in which each twin is aligned with the matrix, E-martensite (hexagonal lattice), and/or  $\alpha'$ -martensite (body centered tetragonal lattice). These transformations may depend upon the specific steel chemistry, strain conditions, and/or temperature, and the extent of metastability may vary. Strain conditions sufficient to induce such phase transformations may be encountered during manufacturing. Service conditions may also be sufficient to promote such phase transformations in some instances.

Sufficient carbon content is present in the austenitic steels of the present disclosure to stabilize the austenite phase. Carbon particularly helps in stabilizing the austenite phase during cooling from the melt and during plastic deformation. Additionally, carbon serves to strengthen the austenitic steels through solid solution strengthening. The carbon content may be chosen such that the solubility of carbon is high in the austenite phase, such as in the form of one or more soluble carbides. Insoluble carbides or free carbon may also be present in some compositions. When the carbon content is too high, significant carbide precipitation can occur during processing and high temperature thermal cycles during chain fabrication. Excessive carbide formation may reduce toughness. For the foregoing reasons, the carbon content in the austenitic steels of the present disclosure may range from about 0.4-0.8 wt. % C. In more specific embodiments, the austenitic steels of the present disclosure may comprise from about 0.5-0.7 wt. % C or from about 0.55-0.65 wt. % C.

Manganese is the primary alloying element in high-manganese steels, such as the austenitic steels disclosed herein. Manganese may particularly aid in stabilizing the austenite phase during cooling and deformation of the austenitic steels. Additionally, the amount of manganese may determine how the austenitic steels respond or trans-

form when strained. At manganese contents greater than about 25 wt. %, the austenite phase may deform via dislocation slip when it is mechanically strained. At manganese contents between about 15 wt. % and about 25 wt. %, the austenite phase is mildly metastable and may undergo twinning during deformation. The twinning may result in a high degree of work hardening and can produce very high tensile strength and uniform elongation. At manganese contents less than about 15 wt. %, the austenite phase is more metastable (less stable) and can transform into an  $\epsilon$ -martensite and/or  $\alpha'$ -martensite phase upon mechanical straining. A combination of twinning and transformation to  $\epsilon$ -martensite may provide a favorable combination of mechanical behavior (strength, toughness, wear resistance, corrosion resistance) for mooring chain applications. For the foregoing reasons, the manganese content in the austenitic steels of the present disclosure may range from about 12-25 wt. % Mn. In more specific embodiments, the austenitic steels of the present disclosure may comprise from about 12-18 wt. % Mn, or from about 14-19 wt. % Mn, or from about 16-20 wt. % Mn. In some embodiments, in addition to a predominant austenite phase, the austenitic steels of the present disclosure may comprise a twinned phase and/or  $\epsilon$ -martensite.

The chromium content in the austenitic steels of the present disclosure may particularly aid in facilitating corrosion resistance. The chromium content may be limited based upon one or more of the following considerations: (1) limiting steel costs by avoiding Cr levels that are too high, (2) limiting austenite phase destabilization for Cr levels that are too high, thereby encouraging ferrite phase formation, and (3) limiting carbide precipitation (and possible toughness loss) during processing and high-temperature thermal cycling for Cr levels that are too high. The chromium content is therefore chosen to convey acceptable corrosion resistance to the austenitic steels without promoting excessive austenite phase destabilization or carbide precipitation. For the foregoing reasons, the chromium content in the austenitic steels of the present disclosure may range from about 4-15 wt. % Cr. In more specific embodiments, the austenitic steels of the present disclosure may comprise from about 5-10 wt. % Cr, or from about 10-15 wt. % Cr.

The silicon content in the austenitic steels of the present disclosure may play one or more of the following roles: serving as a ferrite stabilizer, promoting  $\epsilon$ -martensite formation during ambient temperature deformation, and strengthening the austenite phase through solid solution strengthening. The silicon content may be limited to promote sufficient strengthening without inducing excessive ferrite stabilization. For the foregoing reasons, the silicon content in the austenitic steels of the present disclosure may be present in a non-zero amount up to about 3 wt. % Si. In more specific embodiments, the austenitic steels of the present disclosure may comprise a non-zero amount of silicon up to about 1 wt. % Si. In still more specific embodiments, the austenitic steels of the present disclosure may comprise an amount of silicon ranging from about 0.01 wt. % Si to about 3 wt. % Si, or from about 0.01 wt. % Si to about 1 wt. % Si, or from about 0.01 wt. % Si to about 0.2 wt. % Si.

Aluminum is a ferrite stabilizer, and significant amounts of aluminum can destabilize the austenite phase during cooling. At lower levels, however, aluminum can stabilize the austenite phase to some degree in the austenitic steels of the present disclosure. Stabilization may include action against strain-induced phase transformation taking place during deformation and providing a small amount of solid solution strengthening. For the foregoing reasons, the alu-

minimum content in the austenitic steels of the present disclosure may be present in a non-zero amount up to about 0.5 wt. % Al. In more specific embodiments, the austenitic steels of the present disclosure may comprise a non-zero amount of aluminum up to about 0.1 wt. % Al or up to about 0.08 wt. % Al. In still more specific embodiments, the austenitic steels of the present disclosure may comprise an amount of aluminum ranging from about 0.001 wt. % Al to about 0.5 wt. % Al, or from about 0.001 wt. % Al to about 0.1 wt. % Al, or from about 0.001 wt. % Al to about 0.08 wt. % Al.

Molybdenum is a very effective solid solution strengthener of the austenite phase in the austenitic steels of the present disclosure and may be utilized in small quantities to increase strength. Depending on strength requirements for a mooring chain, the inclusion of molybdenum in the austenitic steel forming the mooring chain may be optional. For the foregoing reasons, according to some embodiments, the molybdenum content in the austenitic steels of the current disclosure may be present in an amount up to about 5 wt. %. The austenitic steels may be substantially molybdenum-free (<0.001 wt. % Mo as a trace impurity) in some embodiments. In more specific embodiments in which molybdenum is present, the austenitic steels of the present disclosure may comprise a non-zero amount of molybdenum up to about 5 wt. %, or up to about 1 wt. %, or up to about 0.5 wt. %, or up to about 0.1 wt. %. In still more specific embodiments, the austenitic steels of the present disclosure may comprise an amount of molybdenum ranging from about 0.001 wt. % Mo to about 5 wt. % Mo, or from about 0.001 wt. % Mo to about 1 wt. % Mo, or from about 0.001 wt. % Mo to about 0.5 wt. % Mo, or from about 0.001 wt. % Mo to about 0.1 wt. % Mo. In other embodiments, the austenitic steels of the present disclosure may comprise between about 0-5 wt. % molybdenum, with the inclusion of molybdenum being optional. In more specific examples, the austenitic steels of the present disclosure may comprise about 0-5 wt. % Mo, or about 0-1 wt. % Mo, or about 0-0.5 wt. % Mo, or about 0-0.1 wt. % Mo.

Nitrogen is an effective solid solution strengthener and a precipitate (nitride) former. In Cr, and Mn alloyed austenitic steels, the nitrogen solubility limit is typically determined by the equilibrium between the matrix and chromium nitride (e.g., Cr<sub>2</sub>N). When the nitrogen concentration is above the solubility limit, the alloyed steel is susceptible to chromium nitride precipitation, especially at temperatures between approximately 500° C. and 1100° C. The kinetics of precipitation are highly composition- and temperature-dependent. The effectiveness of nitrogen as a strengthener is such that if the nitrogen content is too high, hot workability (required for manufacturing) of the austenitic steel may be negatively impacted. For the foregoing reasons, the nitrogen content in the austenitic steels of the current disclosure may be present in a non-zero amount up to about 0.1 wt. % N. In more specific embodiments, the austenitic steels of the present disclosure may comprise a non-zero amount of nitrogen up to about 0.05 wt. % N, or up to about 0.01 wt. % N, or up to 0.008 wt. % N. In still more specific embodiments, the austenitic steels of the present disclosure may comprise an amount of nitrogen ranging from about 0.001 wt. % N to about 0.1 wt. % N, or from about 0.001 wt. % N to about 0.05 wt. % N, or from about 0.001 wt. % N to about 0.01 wt. % N, or from about 0.001 wt. % N to about 0.008 wt. % N. Nitrogen may also lessen corrosion, particularly pitting corrosion, in the austenitic steels. Without being bound by any theory or mechanism, it is believed that the corrosion protection afforded by nitrogen may be due to its influence in stabilizing passivating oxide films and pro-

moting rapid re-passivation in local areas where a passivating oxide film has been disrupted.

Accordingly, mooring chains comprising the austenitic steels described hereinabove may comprise a plurality of links comprising an austenitic steel, which comprises:

0.4-0.8 wt. % C,  
12-25 wt. % Mn,  
4-15 wt. % Cr,  
a non-zero amount of Si<3 wt. % Si,  
a non-zero amount of Al<0.5 wt. % Al,  
a non-zero amount of N<0.1 wt. % N,  
<5 wt. % Mo, and  
balance Fe and inevitable impurities.

According to more specific embodiments, mooring chains of the present disclosure may comprise an austenitic steel comprising carbon in an amount ranging from about 0.5-0.7 wt. % C or from about 0.55-0.65 wt. % C. In more specific embodiments, the foregoing amounts of carbon may be present in the austenitic steel in combination with about 12-25 wt. % Mn, about 4-15 wt. % Cr, a non-zero amount of Si less than about 3 wt. % Si, a non-zero amount of Al less than about 0.5 wt. % Al, a non-zero amount of Mo less than about 5 wt. % Mo or an amount of Mo less than about 5 wt. % Mo, and a non-zero amount of N less than about 0.1 wt. % N, including any sub-range within the foregoing amounts of Mn, Cr, Si, Al, Mo, and N.

According to some more specific embodiments, mooring chains of the present disclosure may comprise an austenitic steel comprising manganese in an amount ranging between about 16-20 wt. %. In more specific embodiments, the foregoing amounts of manganese may be present in the austenitic steel in combination with about 0.4-0.8 wt. % C, about 4-15 wt. % Cr, a non-zero amount of Si less than about 3 wt. % Si, a non-zero amount of Al less than about 0.5 wt. % Al, a non-zero amount of Mo less than about 5 wt. % Mo or an amount of Mo less than about 5 wt. % Mo, and a non-zero amount of N less than about 0.1 wt. % N, including any sub-range within the foregoing amounts of C, Cr, Si, Al, Mo, and N.

According to some more specific embodiments, mooring chains of the present disclosure may comprise an austenitic steel comprising about 5-10 wt. % Cr, or about 8-15 wt. % Cr. In more specific embodiments, the foregoing amounts of chromium may be present in the austenitic steel in combination with about 0.4-0.8 wt. % C, about 12-25 wt. % Mn, a non-zero amount of Si less than about 3 wt. % Si, a non-zero amount of Al less than about 0.5 wt. % Al, a non-zero amount of Mo less than about 5 wt. % Mo or an amount of Mo less than about 5 wt. % Mo, and a non-zero amount of N less than about 0.1 wt. % N, including any sub-range within the foregoing amounts of C, Mn, Si, Al, Mo, and N.

According to some more specific embodiments, mooring chains of the present disclosure may comprise an austenitic steel comprising a non-zero amount of silicon less than about 3 wt. % Si or less than about 1 wt. % Si. In more specific embodiments, the foregoing amounts of silicon may be present in the austenitic steel in combination with about 0.4-0.8 wt. % C, about 12-25 wt. % Mn, about 4-15 wt. % Cr, a non-zero amount of Al less than about 0.5 wt. % Al, a non-zero amount of Mo less than about 5 wt. % Mo or an amount of Mo less than about 5 wt. % Mo, and a non-zero amount of N less than about 0.1 wt. % N, including any sub-range within the foregoing amounts of C, Mn, Cr, Al, Mo, and N.

According to some more specific embodiments, mooring chains of the present disclosure may comprise an austenitic

steel comprising a non-zero amount of aluminum less than about 0.5 wt. % Al or a non-zero amount of aluminum less than about 0.08 wt. % Al. In more specific embodiments, the foregoing amounts of aluminum may be present in the austenitic steel in combination with about 0.4-0.8 wt. % C, about 12-25 wt. % Mn, about 4-15 wt. % Cr, a non-zero amount of Si less than about 3 wt. % Si, a non-zero amount of Mo less than about 5 wt. % Mo or an amount of Mo less than about 5 wt. % Mo, and a non-zero amount of N less than about 0.1 wt. % N, including any sub-range within the foregoing amounts of C, Mn, Cr, Si, Mo, and N.

According to some more specific embodiments, mooring chains of the present disclosure may comprise an austenitic steel comprising a non-zero amount of molybdenum less than about 5 wt. % Mo or an amount of Mo less than about 5 wt. % Mo. In more specific embodiments, the foregoing amounts of molybdenum may be present in the austenitic steel in combination with about 0.4-0.8 wt. % C, about 12-25 wt. % Mn, about 4-15 wt. % Cr, a non-zero amount of Si less than about 3 wt. % Si, a non-zero amount of Al less than about 0.5 wt. % Al, and a non-zero amount of N less than about 0.1 wt. % N, including any sub-range within the foregoing amounts of C, Mn, Cr, Si Al, and N.

According to some more specific embodiments, mooring chains of the present disclosure may comprise an austenitic steel comprising a non-zero amount of nitrogen less than about 0.1 wt. % N, or a non-zero amount of nitrogen less than about 0.008 wt. % N. In more specific embodiments, the foregoing amounts of nitrogen may be present in the austenitic steel in combination with about 0.4-0.8 wt. % C, about 12-25 wt. % Mn, about 4-15 wt. % Cr, a non-zero amount of Si less than about 3 wt. % Si, a non-zero amount of Al less than about 0.5 wt. % Al, and a non-zero amount of Mo less than about 5 wt. % Mo or an amount of Mo less than about 5 wt. % Mo, including any sub-range within the foregoing amounts of C, Mn, Cr, Si, Al, and Mo.

Moreover, in any of the foregoing austenitic steels, the austenitic steel may comprise at least 0.01 wt. % Si, at least 0.001 wt. % Al, and at least 0.001 wt. % N. Optionally, at least 0.001 wt. % Mo may also be present.

In various embodiments, mooring chains comprising the austenitic steels of the present disclosure may feature a grain size ranging from about 20 microns to about 200 microns, or any subrange thereof.

Mooring chains of the present disclosure may feature an austenitic steel having one or more of the following physical properties: a yield strength of at least 440 MPa and an ultimate tensile strength of at least about 990 MPa, a corrosion rate ranging at 25° C. and 1 bar pressure of about 0.2 mils per year (mpy) to about 0.7 mpy, is Charpy notch impact toughness at -20° C. of about 80 J to about 220 J, and an ASTM G99 wear value characterized by an average pin loss measurement of about 2 mg or less and an average disk mass loss measurement of 8 mg or less.

According to some embodiments, mooring chains of the present disclosure may feature links that are joined together using butt welding techniques. Both studded and studless links may be formed.

In some embodiments, mooring chains of the present disclosure may be adapted for exposure to multiple conditions. In particular, such mooring chains may feature chain links in a first section adapted for continuous or near-continuous exposure to seawater and chain lengths in a second section adapted for limited or no exposure to seawater, wherein the chain lengths in each section may comprise different steel compositions. In more specific embodiments, such mooring chains may comprise a top chain

coupled to a bottom chain, in which the top chain resides above an anticipated water line or splash zone in a moored offshore structure and the bottom chain resides in a splash zone or below an anticipated water line of the moored offshore structure. In such mooring chains, the top chain may comprise a ferritic carbon steel and the bottom chain may comprise an austenitic steel of the present disclosure. In other embodiments, the top chain and the bottom chain may comprise austenitic steels of the present disclosure, each having different compositions. In still other embodiments, the top chain may comprise an austenitic steel of the present disclosure, and the bottom chain may comprise a ferritic carbon steel. The austenitic steels of the present disclosure may be particularly advantageous as a top chain that is periodically exposed to water and/or is in a region a few meters below the water line. Steels in the foregoing regions (e.g., in splash zones or just below the water line) may be especially susceptible to corrosion, which may be mitigated through use of the austenitic steels described herein.

In addition to mooring chains comprising the austenitic steels disclosed herein, the present disclosure also contemplates other structures comprising the austenitic steels that may be continuously or periodically in contact with a seawater environment. Such structures may include, for example, platform legs, risers, boat hulls, pipelines, and the like.

The present disclosure also provides moored offshore structures that are held in place by one or more mooring chains of the present disclosure. Any of the austenitic steels disclosed herein may be used for forming mooring chains suitable for securing a particular type of floating offshore structure. Illustrative floating offshore structures that may be held in place with the mooring chains of the present disclosure include, for example, oil drilling and production platforms, buoys, floating storage and offloading vessels (FSO-vessels), drilling ships, offshore wind turbines, and the like. Choice of a mooring chain suitable for a given application may depend upon the type of floating offshore structure being moored, and the particular environmental conditions present at the site of mooring.

In some or other more specific embodiments, the mooring chains of the present disclosure may be prepared from an austenitic steel that has been processed using a hot rolling procedure that comprises: hot rolling the austenitic steel in a series of hot rolling cycles, each cycle having a progressively decreasing temperature, thereby forming an austenitic steel sheet; wherein the austenitic steel sheet is decreased in thickness by about 10% to about 25% during each hot rolling cycle; and after a final hot rolling cycle, cooling the austenitic steel sheet to room temperature under a water curtain. The austenitic steel provided to the first hot rolling cycle may be in the form of an austenitic steel ingot.

The mooring chains disclosed herein can be particularly useful in securing a floating offshore structure by transferring loading forces imposed upon the floating offshore structure, through the mooring chain, and to a rigid pile anchor which is secured to the earthen surface below the body of water. The mooring chain may be a component part of a flexible connection connecting the floating offshore structure to the rigid pile anchor or may be the sole component of the flexible connection. The mooring chains herein are particularly useful in reducing corrosion rates experienced due to stresses imposed on the mooring chain, particularly in a sea water environment and/or wherein the mooring chain is located in a periodic splash zone, wherein the portion of the mooring chain is periodically submerged under the body of water and periodically

## 11

exposed to air above the body of water. In this splash zone, the austenitic steel of the mooring chains can have a corrosion rate of about 0.2 to about 0.7 mils per year (mpy). The mooring chains herein may be to be utilized as bare (i.e., no coatings applied to the chain) in service and maintain very low material loss due to corrosive effects.

Embodiments disclosed herein include: A. Mooring chains. The mooring chains comprise: a plurality of links comprising an austenitic steel, the austenitic steel comprising:

0.4-0.8 wt. % C,  
12-25 wt. % Mn,  
4-15 wt. % Cr,  
a non-zero amount of Si<3 wt. % Si,  
a non-zero amount of Al<0.5 wt. % Al,  
a non-zero amount of N<0.1 wt. % N,  
<5 wt. % Mo, and  
balance Fe and inevitable impurities.

Embodiment A may have one or more of the following additional elements in any combination:

Element 1: wherein the austenitic steel comprises a non-zero amount of Si<1 wt. % Si.

Element 2: wherein the austenitic steel comprises 0.5-0.7 wt. % C.

Element 3: wherein the austenitic steel comprises 0.55-0.65 wt. % C.

Element 4: wherein the austenitic steel comprises 16-20 wt. % Mn.

Element 5: wherein the austenitic steel comprises a non-zero amount of Al<0.08 wt. % Al.

Element 6: wherein the austenitic steel comprises a non-zero amount of N<0.008 wt. % N.

Element 7: wherein the austenitic steel comprises at least 0.01 wt. % Si, at least 0.001 wt. % Al, and at least 0.001 wt. % N.

Element 8: wherein the austenitic steel comprises 5-10 wt. % Cr.

Element 9: wherein the austenitic steel comprises 8-15 wt. % Cr.

Element 10: wherein the austenitic steel comprises a non-zero amount of Mo<5 wt. % Mo.

Element 11: wherein the austenitic steel has a yield strength of at least about 440 MPa and an ultimate tensile strength of at least about 990 MPa.

Element 12: wherein the austenitic steel has a corrosion rate at 25° C. and 1 bar pressure of about 0.2 to about 0.7 mils per year (mpy).

Element 13: wherein the austenitic steel has a Charpy notch impact toughness at -20° C. of about 80 J to about 220 J.

Element 14: wherein the austenitic steel has an ASTM G99 wear value characterized by an average pin loss measurement of 2 mg or less and an average disk mass loss measurement of 8 mg or less.

Element 15: wherein each link is butt welded together.

Element 16: wherein the mooring chain comprises a top chain coupled to a bottom chain, the top chain configured for residing above an anticipated water line and the bottom chain configured for residing below an anticipated water line, the top chain and the bottom chain differing compositionally from one another and at least one of the top chain and the bottom chain comprising the austenitic steel.

Element 17: wherein the austenitic steel is processed by a hot rolling procedure, the hot rolling procedure comprising: hot rolling a steel ingot in a series of hot rolling cycles, each cycle having a progressively decreasing temperature, thereby forming an austenitic steel sheet; wherein the aus-

## 12

tenitic steel sheet is decreased in thickness by about 10% to about 25% during each hot rolling cycle; and after a final hot rolling cycle, cooling the austenitic steel sheet to room temperature under a water curtain.

By way of non-limiting example, exemplary combinations include: The mooring chain of A in combination with elements 1 and 10; 2 and 10; 3 and 10; 4 and 10; 5 and 10; 6 and 10; 7 and 10; 8 and 10; 9 and 10; 10 and 11; 10 and 12; 10 and 13; 10 and 14; 10 and 15; 10 and 16; and 10 and

17. The mooring chain of A in combination with elements 1 and 2; 1 and 3; 1 and 4; 1 and 5; 1 and 6; 1 and 7; 1 and 8; 1 and 9; 1 and 11; 1 and 12; 1 and 13; 1 and 14; 1 and 15; 1 and 16; 1 and 17; 2 and 4; 2 and 5; 2 and 6; 2 and 7; 2 and 8; 2 and 9; 2 and 11; 2 and 12; 2 and 13; 2 and 14; 2 and 15; 2 and 16; 2 and 17; 3 and 5; 3 and 6; 3 and 7; 3 and 8; 3 and 9; 3 and 11; 3 and 12; 3 and 13; 3 and 14; 3 and 15; 3 and 16; 3 and 17; 4 and 5; 4 and 6; 4 and 7; 4 and 8; 4 and 9; 4 and 11; 4 and 12; 4 and 13; 4 and 14; 4 and 15; 4 and 16; 4 and 17; 5 and 6; 5 and 7; 5 and 8; 5 and 9; 5 and 11; 5 and 12; 5 and 13; 5 and 14; 5 and 15; 5 and 16; 5 and 17; 6 and 7; 6 and 8; 6 and 9; 6 and 11; 6 and 12; 6 and 13; 6 and 14; 6 and 15; 6 and 16; 6 and 17; 7 and 8; 7 and 9; 7 and 11; 7 and 12; 7 and 13; 7 and 14; 7 and 15; 7 and 16; 7 and 17; 8 and 11; 8 and 12; 8 and 13; 8 and 14; 8 and 15; 8 and 16; 8 and 17; 9 and 11; 9 and 12; 9 and 13; 9 and 14; 9 and 15; 9 and 16; 9 and 17; 11 and 12; 11 and 13; 11 and 14; 11 and 15; 11 and 16; 11 and 17; 12 and 13; 12 and 14; 12 and 15; 12 and 16; 12 and 17; 13 and 14; 13 and 15; 13 and 16; 13 and 17; 14 and 15; 14 and 16; 14 and 17; 15 and 16; 15 and 17; and 16 and 17, any of which may be in further combination with element 10. The mooring chain of A in combination with elements 1, 2 and 4; 1, 2 and 5; 1, 2 and 6; 1, 2 and 7; 1, 2 and 8; 1, 2 and 9; 1, 2 and 10; 2, 4 and 5; 2, 4 and 6; 2, 4, 5 and 6; 2, 4, 5 and 7; 2, 4-6 and 7; 2, 4, 5 and 8; 2, 4, 5 and 9; 2, 4, 6 and 9; 2, 4-6 and 8; 2, 4-6 and 9; 2, 4 and 5-8; 2, 4, 5-7 and 9; 2, 5 and 6; 2, 5 and 7; 2 and 5-7; 2, 5-7 and 8; 2, 5-7 and 9; 2, 6 and 7; 2 and 6-8; 2, 6, 7 and 9; 2, 7 and 8; 2, 7 and 9; 4-6; 4, 5 and 7; 4-7; 4, 5 and 8; 4, 5 and 9; 4, 5, 7 and 8; 4, 5, 7 and 9; 4, 6 and 7; 4, 6 and 8; 4, 6 and 9; 4 and 6-8; 4, 6, 7 and 9; 5-7; 5-8; 5-7 and 9; 6-8; and 6, 7 and 9, any of which may be in further combination with element 10 and/or in further combination with one or

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 83

TABLE 1

| Alloy           | C     | Si    | Mn     | Al    | Cr     | Mo   | N      | Ni   | Co  |
|-----------------|-------|-------|--------|-------|--------|------|--------|------|-----|
| 1               | 0.6   | 0.109 | 18.6   | 0.059 | 5.09   | —    | 0.0072 | —    | —   |
| 2               | 0.591 | 0.098 | 18.084 | 0.059 | 10.269 | —    | 0.0076 | —    | —   |
| 3               | 0.562 | 2.871 | 16.77  | 0.051 | 5.259  | —    | 0.005  | —    | —   |
| 4 (Comparative) | 0.096 | —     | 1.6    | —     | 1.0    | 0.35 | —      | 1.0  | 0.6 |
| 5 (Comparative) | <0.2  | —     | 2.6    | —     | 0.36   | —    | —      | 0.57 | 0.6 |

The inventive steel alloys were initially produced in a 5 inch thick ingot form. The initially produced ingot was hot rolled in progressively decreasing temperature steps between 1150° C. and 843° C., with a thickness reduction of 15-20% taking place at each hot rolling stage. Table 2 shows a representative schedule of the hot rolling conditions at each stage.

10 strength values exhibited by Alloys 1-3 are indicative of work hardenability, which is beneficial in mooring chain applications. The work hardenability is believed to be due to micro-twinning and E-martensite formation upon plastic deformation.

15 FIG. 1 shows a chart displaying Charpy V-Notch (CVN) impact toughness testing data for Alloys 1-3 of the present

TABLE 2

| Pass #    | Pre-Step Temperature (° C.)                                                                                                 | PreStep Thickness (in.) | Post Step Thickness (in.) | Reduction (%) |
|-----------|-----------------------------------------------------------------------------------------------------------------------------|-------------------------|---------------------------|---------------|
| Reheating | 1150                                                                                                                        | —                       | —                         | —             |
| 1         | 1121                                                                                                                        | 5.00                    | 4.25                      | 15            |
| 2         | 1079                                                                                                                        | 4.25                    | 3.61                      | 15            |
| 3         | 1038                                                                                                                        | 3.61                    | 3.07                      | 15            |
| 4         | 1010                                                                                                                        | 3.07                    | 2.46                      | 20            |
| 5         | 982                                                                                                                         | 2.46                    | 1.97                      | 20            |
| 6         | 954                                                                                                                         | 1.97                    | 1.57                      | 20            |
| 7         | 927                                                                                                                         | 1.57                    | 1.26                      | 20            |
| 8         | 885                                                                                                                         | 1.26                    | 1.01                      | 20            |
| 9         | 843                                                                                                                         | 1.01                    | 0.80                      | 20            |
| Quench    | Cooling to room temperature starts immediately after finishing the rolling operation and takes place under a water curtain. |                         |                           |               |

The yield and tensile strengths of the steel alloys shown in Table 1 were evaluated under standard conditions using ASTM E8 testing methods at room temperature. Testing results are shown in Table 3. Yield and tensile strengths for IACS steel grades R3, R3S and R4 are also included in Table 3 for reference. The values represent the range of two tested samples.

35 disclosure. Testing was conducted under standard conditions using ASTM A370 testing method at -20° C. As shown, the CVN impact toughness was greatest for Alloy 1. In addition, Alloys 1-3 all exhibited CVN impact toughness values greater than those shown by the IACS alloys. The chart also shows the (CVN) impact toughness testing data for IACS Grades R3, R3S and R4 for comparison.

40 FIG. 2 shows a chart displaying ASTM G99 pin and disk average mass loss measurements for Alloys 1-3 of the present disclosure and Comparative Alloy 4 in a synthetic seawater environment (ASTM D1141 synthetic seawater). The pin and disk mass loss measurements are characteristic of wear performance upon field deployment. As shown, Alloys 1-3 all exhibited much smaller mass losses on both 45 the pin and the disk portions relative to Comparative Alloy 4 under the standard testing conditions. The pin mass loss portion for Alloys 1-3 was much smaller than the disk mass loss portion. In contrast, Comparative Alloy 4 exhibited a pin mass loss portion that was much higher than the disk 50 mass loss portion. The small pin mass loss portion of Alloys 1-3 is believed to be due to surface work hardening taking place upon the pin throughout the test.

55 FIG. 3 shows a chart displaying steady state corrosion data for Alloys 1-3 of the present disclosure relative to Comparative Alloys 4 and 5 in a synthetic seawater environment at 25° C. and 1 bar pressure. The testing duration was one week. The synthetic seawater had the following composition: NaCl (26.25 g/L), KCl (0.6 g/L), CaCl<sub>2</sub>·2H<sub>2</sub>O (1.5 g/L), MgCl<sub>2</sub>·6H<sub>2</sub>O (5.7 g/L), MgSO<sub>4</sub>·7H<sub>2</sub>O (6.75 g/L) and NaHCO<sub>3</sub> (0.17 g/L). As shown, Alloys 1-3 exhibited 60 significantly different steady state corrosion rates relative to Comparative Alloys 4 and 5. The corrosion rates for Alloys 65

As shown in Table 3, Alloy 1 and Comparative Alloy 4 had comparable yield strength values, but Alloy 1 had a significantly greater ultimate tensile strength. Alloys 2 and 3 likewise had comparable yield strengths to Comparative Alloy 5 but significantly greater ultimate tensile strength values. The yield strength values for Alloys 1-3 spanned the range of yield strengths for IACS Grade R3, R3S and R4. The high yield strength values are believed to be due to solid solution strengthening of the austenite phase in the steel alloys disclosed herein. The ultimate tensile strength values of Alloys 1-3 were also all significantly greater than those exhibited by the IACS alloys. The high ultimate tensile

1-3 varied from 0.2-0.7 mils per year (mpy), in comparison to rates of 3.0-3.5 mpy for Comparative Alloys 4 and 5. Alloy 2, which contained a higher percentage of Cr, exhibited better corrosion resistance than did Alloys 1 and 3, whose Cr contents were lower.

FIGS. 4A-4E show corresponding cyclic polarization curves for Alloys 1-3 and Comparative Alloys 4 and 5 in a synthetic seawater environment. Testing was conducted as above. The narrow cyclic polarization curves for Comparative Alloys 4 and 5 (FIGS. 4D and 4E) relative to the wider cyclic polarization curves of Alloys 1-3 (FIGS. 4A-4C) showed that Alloys 1-3 were more corrosion resistant. In addition, the polarization curves for Alloys 1-3 showed some signs of protective passivation behavior, whereas the polarization curves for Comparative Alloys 4 and 5 did not.

All documents described herein are incorporated by reference herein for purposes of all jurisdictions where such practice is allowed, including any priority documents and/or testing procedures to the extent they are not inconsistent with this text. As is apparent from the foregoing general description and the specific embodiments, while forms of the disclosure have been illustrated and described, various modifications can be made without departing from the spirit and scope of the disclosure. Accordingly, it is not intended that the disclosure be limited thereby. For example, the compositions described herein may be free of any component, or composition not expressly recited or disclosed herein. Any method may lack any step not recited or disclosed herein. Likewise, the term "comprising" is considered synonymous with the term "including." Whenever a method, composition, element or group of elements is preceded with the transitional phrase "comprising," it is understood that we also contemplate the same composition or group of elements with transitional phrases "consisting essentially of," "consisting of," "selected from the group of consisting of," or "is" preceding the recitation of the composition, element, or elements and vice versa.

Unless otherwise indicated, all numbers expressing quantities of ingredients, properties such as molecular weight, reaction conditions, and so forth used in the present specification and associated claims are to be understood as being modified in all instances by the term "about." Accordingly, unless indicated to the contrary, the numerical parameters set forth in the following specification and attached claims are approximations that may vary depending upon the desired properties sought to be obtained by the embodiments of the present invention. At the very least, and not as an attempt to limit the application of the doctrine of equivalents to the scope of the claim, each numerical parameter should at least be construed in light of the number of reported significant digits and by applying ordinary rounding techniques.

Whenever a numerical range with a lower limit and an upper limit is disclosed, any number and any included range falling within the range is specifically disclosed. In particular, every range of values (of the form, "from about a to about b," or, equivalently, "from approximately a to b," or, equivalently, "from approximately a-b") disclosed herein is to be understood to set forth every number and range encompassed within the broader range of values. Also, the terms in the claims have their plain, ordinary meaning unless otherwise explicitly and clearly defined by the patentee. Moreover, the indefinite articles "a" or "an," as used in the claims, are defined herein to mean one or more than one of the element that it introduces.

One or more illustrative embodiments are presented herein. Not all features of a physical implementation are described or shown in this application for the sake of clarity.

It is understood that in the development of a physical embodiment of the present disclosure, numerous implementation-specific decisions must be made to achieve the developer's goals, such as compliance with system-related, business-related, government-related and other constraints, which vary by implementation and from time to time. While a developer's efforts might be time-consuming, such efforts would be, nevertheless, a routine undertaking for one of ordinary skill in the art and having benefit of this disclosure.

Therefore, the present disclosure is well adapted to attain the ends and advantages mentioned as well as those that are inherent therein. The particular embodiments disclosed above are illustrative only, as the present disclosure may be modified and practiced in different but equivalent manners apparent to one having ordinary skill in the art and having the benefit of the teachings herein. Furthermore, no limitations are intended to the details of construction or design herein shown, other than as described in the claims below. It is therefore evident that the particular illustrative embodiments disclosed above may be altered, combined, or modified and all such variations are considered within the scope and spirit of the present disclosure. The embodiments illustratively disclosed herein suitably may be practiced in the absence of any element that is not specifically disclosed herein and/or any optional element disclosed herein.

What is claimed is:

1. A mooring chain comprising:  
a plurality of links comprising an austenitic steel, the austenitic steel comprising:

0.4-0.8 wt. % C,

12-25 wt. % Mn,

4-15 wt. % Cr,

a non-zero amount of Si<3 wt. % Si,

a non-zero amount of Al<0.5 wt. % Al,

a non-zero amount of N<0.1 wt. % N,

<5 wt. % Mo, and

balance Fe and inevitable impurities;

wherein the austenitic steel has a corrosion rate at 25° C. and 1 bar pressure of about 0.2 to about 0.7 mils per year (mpy).

2. The mooring chain of claim 1, wherein the austenitic steel comprises a non-zero amount of Si<1 wt. % Si.

3. The mooring chain of claim 1, wherein the austenitic steel comprises 0.55-0.65 wt. % C.

4. The mooring chain of claim 1, wherein the austenitic steel comprises 16-20 wt. % Mn.

5. The mooring chain of claim 1, wherein the austenitic steel comprises a non-zero amount of Al<0.08 wt. % Al.

6. The mooring chain of claim 1, wherein the austenitic steel comprises a non-zero amount of N<0.008 wt. % N.

7. The mooring chain of claim 1, wherein the austenitic steel comprises at least 0.01 wt. % Si, at least 0.001 wt. % Al, and at least 0.001 wt. % N.

8. The mooring chain of claim 1, wherein the austenitic steel comprises 5-10 wt. % Cr.

9. The mooring chain of claim 1, wherein the austenitic steel comprises a non-zero amount of Mo<5 wt. % Mo.

10. The mooring chain of claim 1, wherein the austenitic steel has a yield strength of at least about 440 MPa and an ultimate tensile strength of at least about 990 MPa.

11. The mooring chain of claim 1, wherein the austenitic steel has a Charpy notch impact toughness at -20° C. of about 80 J to about 220 J.

12. The mooring chain of claim 1, wherein the austenitic steel has an ASTM G99 wear value characterized by an average pin loss measurement of 2 mg or less and an average disk mass loss measurement of 8 mg or less.

**17**

13. The mooring chain of claim 1, wherein the mooring chain comprises a top chain coupled to a bottom chain, the top chain configured for residing above an anticipated water line and the bottom chain configured for residing below an anticipated water line, the top chain and the bottom chain differing compositionally from one another and at least one of the top chain and the bottom chain comprising the austenitic steel.

14. The mooring chain of claim 1, wherein the austenitic steel is processed by a hot rolling procedure, the hot rolling procedure comprising:

hot rolling a steel ingot in a series of hot rolling cycles, each cycle having a progressively decreasing temperature, thereby forming an austenitic steel sheet; wherein the austenitic steel sheet is decreased in thickness by about 10% to about 25% during each hot rolling cycle; and after a final hot rolling cycle, cooling the austenitic steel sheet to room temperature under a water curtain.

15. A process for mooring a floating offshore structure, comprising:

providing at least one flexible connection between a floating offshore structure located on a body of water and a rigid pile anchor located in a body of water, wherein the rigid pile anchor is secured to the earthen surface located below the body of water;

maintain the position of the floating offshore structure on the body of water through the use of the flexible connection by transferring loading forces imposed upon the floating offshore structure, through the flexible connection and to the rigid pile anchor;

5

10

15

20

25

30

**18**

wherein the flexible connection is comprised of a mooring chain, such mooring chain comprising:

a plurality of links comprising an austenitic steel, the austenitic steel comprising:

0.4-0.8 wt. % C,

12-25 wt. % Mn,

4-15 wt. % Cr,

a non-zero amount of Si<3 wt. % Si,

a non-zero amount of Al<0.5 wt. % Al,

a non-zero amount of N<0.1 wt. % N,

<5 wt. % Mo, and

balance Fe and inevitable impurities;

wherein:

the mooring chain is bare;

at least a portion of the mooring chain is located in a periodic splash zone, wherein the portion of the mooring chain is periodically submerged under the body of water and periodically exposed to air above the body of water; and the body of water is sea water; and the austenitic steel in the periodic splash zone has a corrosion rate of about 0.2 to about 0.7 mils per year (mpy).

16. The process of claim 15, wherein the austenitic steel has a yield strength of at least about 440 MPa and an ultimate tensile strength of at least about 990 MPa; and the austenitic steel has a Charpy notch impact toughness at -20° C. of about 80 J to about 220 J.

17. The process of claim 15, wherein the austenitic steel has an ASTM G99 wear value characterized by an average pin loss measurement of 2 mg or less and an average disk mass loss measurement of 8 mg or less.

\* \* \* \* \*